



US012071728B2

(12) **United States Patent**  
Oishi et al.

(10) **Patent No.:** US 12,071,728 B2  
(45) **Date of Patent:** Aug. 27, 2024

(54) **METHOD FOR MANUFACTURING PAPER BARRIER BASE MATERIAL**

2010/0239763 A1 9/2010 Åsmus et al.  
2016/0222592 A1\* 8/2016 Müller ..... D21H 23/44  
2019/0270289 A1\* 9/2019 Okamoto ..... B32B 27/00

(71) Applicants: **NIPPON PAPER INDUSTRIES CO., LTD.**, Tokyo (JP); **JUJO THERMAL OY**, Kauttua (FI)

FOREIGN PATENT DOCUMENTS

(72) Inventors: **Yuri Oishi**, Tokyo (JP); **Kenta Watanabe**, Tokyo (JP); **Satoshi Tsuda**, Tokyo (JP); **Masashi Okamoto**, Kauttua (FI); **Hiroshi Koyamoto**, Tokyo (JP)

|    |                    |                          |
|----|--------------------|--------------------------|
| CN | 103476992 A        | 12/2013                  |
| JP | S5474761 A         | 6/1979                   |
| JP | S5485811 A         | 7/1979                   |
| JP | H06294099 A        | 10/1994                  |
| JP | 2009034563 A       | 2/2009                   |
| JP | 2009214373 A       | 9/2009                   |
| JP | 2010529316 A       | 8/2010                   |
| JP | 2011020352 A       | 2/2011                   |
| JP | 2012207319 A       | 10/2012                  |
| JP | 5759449 B2 *       | 8/2015 ..... D21H 17/63  |
| JP | 2015182327 A       | 10/2015                  |
| WO | 2012133092 A1      | 10/2012                  |
| WO | 2017170462 A1      | 10/2017                  |
| WO | WO-2017170462 A1 * | 10/2017 ..... B32B 27/00 |

(73) Assignees: **NIPPON PAPER INDUSTRIES CO., LTD.**, Tokyo (JP); **JUJO THERMAL OY**, Kauttua (FI)

(\*) Notice: Subject to any disclaimer, the term of this patent is extended or adjusted under 35 U.S.C. 154(b) by 292 days.

OTHER PUBLICATIONS

(21) Appl. No.: **17/598,618**

International Search Report (ISR) mailed Jun. 9, 2020, issued for

(22) PCT Filed: **Mar. 27, 2020**

International application No. PCT/JP2020/013898. (2 pages).

(86) PCT No.: **PCT/JP2020/013898**

International Preliminary Report on Patentability, dated Sep. 28, 2021, for corresponding international application PCT/JP2020/013898 (1 page).

§ 371 (c)(1),

Notification Concerning Transmittal of International Preliminary Report on Patentability, mailed Oct. 14, 2021, for corresponding international application PCT/JP2020/013898 (1 page).

(2) Date: **Sep. 27, 2021**

Notification of Transmittal of Translation of the International Preliminary Report on Patentability, mailed Oct. 14, 2021, for corresponding international application PCT/JP2020/013898 (1 page).

(87) PCT Pub. No.: **WO2020/203721**

Written Opinion of the International Searching Authority, mailed Jun. 9, 2020, for corresponding international application PCT/JP2020/013898 (6 page).

PCT Pub. Date: **Oct. 8, 2020**

Extended European Search Report (EESR) dated Nov. 28, 2022, issued for European counterpart patent application No. EP20784310.3 (8 pages).

(65) **Prior Publication Data**

US 2022/0213652 A1 Jul. 7, 2022

Abstract of Larson, R. G. "Spinnability and viscoelasticity." Journal of NonNewtonian Fluid Mechanics 12.3 (1983): 303-315 (1 page). Bengtsson, Jenny, et al. "The challenge of predicting spinnability: Investigating benefits of adding lignin to cellulose solutions in air-gap spinning." Journal of Applied Polymer Science 138.26 (2021): 50629.(10 pages).

(30) **Foreign Application Priority Data**

Mar. 29, 2019 (JP) ..... 2019-067070  
Mar. 29, 2019 (JP) ..... 2019-067071

Bollstrom, Roger, et al. "Barrier properties created by dispersion coating." Tappi J 12.4 (2013): 45-51. (7 pages).

(51) **Int. Cl.**

**D21H 21/16** (2006.01)  
**D21H 19/36** (2006.01)  
**D21H 19/82** (2006.01)  
**D21H 23/48** (2006.01)  
**D21H 27/10** (2006.01)

Griskey, R. Polymer process engineering. Springer Science & Business Media, 1995 (4 pages).

(Continued)

(52) **U.S. Cl.**

CPC ..... **D21H 21/16** (2013.01); **D21H 19/36** (2013.01); **D21H 19/82** (2013.01); **D21H 23/48** (2013.01); **D21H 27/10** (2013.01)

(58) **Field of Classification Search**

CPC ..... D21H 21/16; D21H 19/36; D21H 19/86  
IPC ..... D21H 21/16,19/36, 19/82  
See application file for complete search history.

*Primary Examiner* — Dah-Wei D. Yuan

*Assistant Examiner* — Kristen A Dagenais

(74) *Attorney, Agent, or Firm* — Law Office of Katsuhiro Arai

(56) **References Cited**

U.S. PATENT DOCUMENTS

2004/0121079 A1\* 6/2004 Urscheler ..... D21H 19/82  
427/420  
2007/0037725 A1\* 2/2007 Noerenberg ..... C08G 65/329  
510/421

A method for manufacturing a paper barrier base material includes a step of applying a water vapor barrier layer coating liquid that contains at least a water vapor barrier resin and a pigment onto a paper base material by a curtain coating method to form a water vapor barrier layer. The water vapor barrier layer coating liquid has a spinnability of 0.07 seconds or more and 0.4 seconds or less at a solid content concentration of 32% by weight and a temperature of 25° C. The method is intended to achieve good stability of a coating liquid and good continuous operability.

(56)

**References Cited**

OTHER PUBLICATIONS

- Pizzi, Antonio, and Kashmiri Lal Mittal, eds. Wood adhesives. Zeist, The Netherlands: VSP, 2010 (3 pages).
- Polyvinyl alcohol—Wikipedia (retrieved on Jun. 26, 2023) (3 pages).
- Third Party Observation dated Jul. 3, 2023, issued for European counterpart patent application No. EP20784310.3 (9 pages).

\* cited by examiner

## METHOD FOR MANUFACTURING PAPER BARRIER BASE MATERIAL

### CROSS-REFERENCE TO RELATED APPLICATIONS

This application is the U.S. National Phase under 35 U.S.C. § 371 of International Application PCT/JP2020/013898, filed Mar. 27, 2020, which claims priority to Japanese Patent Application No. JP2019-067070, filed Mar. 29, 2019 and No. JP 2019-067071, filed Mar. 29, 2019. The International Application was published under PCT Article 21(2) in a language other than English.

### TECHNICAL FIELD

The present invention relates to a method for manufacturing a paper barrier base material, in which good stability of a coating liquid and good continuous operability are achieved.

### BACKGROUND ART

A blade coating method and a roll coating method, which are contact coating methods, are generally used for manufacturing a coating layer.

These contact coating methods have the following features in terms of quality.

The blade coating method is leveling coating (smoothing coating) in which a coating liquid is applied to base paper and an excess coating liquid is then scraped off with a blade to achieve a desired coating quantity, and is a so-called post-metered coating method. Therefore, although the surface of the coating layer has good smoothness, a mottled coating surface is likely to be formed because the coating quantity is affected by irregularities of the base paper. In particular, if the base paper has significant irregularities, the coating liquid is scraped off to such an extent that fibers are exposed at protrusions of the base paper because the surface of the base paper is scratched by a blade. In the coating layer formed by the blade coating method, a difference in layer thickness, which is the distance from the surface of the coating layer to the surface of the base paper, is generated due to such variations in coating quantity. Accordingly, there are problems in that variations in performance depending on the layer thickness are generated and that an internal structure is disordered during scraping, and a predetermined performance is not exhibited. In addition, when the coating liquid passes through the blade, the coating liquid is pressurized by the blade, and water in the coating liquid penetrates into paper. When this water is dried, the paper contracts to cause streaky unevenness, and surface texture of the coating surface may be degraded.

On the other hand, the roll coating method is a so-called pre-metered coating method in which coating is performed by transferring, to base paper, a coating liquid that is metered on a roll in advance. Therefore, there is a problem in that it is necessary to uniformly spread in advance a desired amount of coating liquid over a roll, and a complex machine and operations are required. Furthermore, a streaky pattern is likely to be formed during coating, and it is very difficult to obtain a coating surface without coating unevenness. Thus, the viscosity and the concentration of a coating liquid that can be used are limited. In addition, if foreign matter is mixed on the roll that transfers the coating liquid, there is a concern that a portion of the coating liquid on the roll is not transferred to the base paper.

In addition, an operational feature of these contact coating methods is that the operation efficiency is limited. Specifically, in the contact coating methods, since a blade or a roll comes in contact with base paper with a coating liquid therebetween, a large load is applied to the base paper, and paper breakage is highly likely to occur. This tendency increases as the coating speed increases, and the frequency of paper breakage significantly increases. Furthermore, wear of equipment that contacts during coating, i.e., a blade or a roll, is unavoidable, and it is necessary to periodically replace the equipment as consumables. In addition, in the contact coating methods, since the coating equipment is continuously in contact with a coating liquid, dirt is likely to adhere to the coating equipment, and periodical cleaning is necessary in order to suppress the occurrence of coating defects due to the dirt. As described above, the operation efficiency of the contact coating methods is limited. In particular, there is a problem in that the efficiency deteriorates as the coating speed increases.

In contrast to the contact coating methods described above, non-contact coating methods such as a curtain coating method and a spray coating method are known.

The curtain coating method is a coating method in which a coating layer is formed on base paper by forming a curtain film of a coating liquid and passing base paper through the film, and the equipment does not contact the base paper at all during coating. Therefore, in terms of quality, a uniform coating quantity in the width direction and the flow direction is achieved by forming a uniform curtain film of the coating liquid. Because of the non-contact method, the coating liquid can be transferred to the base paper without pressing, a coating layer with a uniform thickness is obtained, and good coatability on the base paper is also achieved. As described above, since a coating layer with a uniform layer thickness is obtained by the curtain coating method, this method is advantageous in that variations in performance depending on the layer thickness are small, and the performance as designed is easily exhibited. In terms of operation, paper breakage during coating is reduced, and no consumables are generated. In addition, the curtain coating method is a pre-metered coating method, in which all the dropped coating liquid is transferred to the base paper. Therefore, it is easy to manage the coating quantity, and coating can be performed in a desired coating quantity by managing the concentration and the flow rate.

As described above, the curtain coating method is a very good coating method, and the application of the curtain coating method to, for example, wax coating on pressure-sensitive copying paper (Patent Literature 1), thermal paper (Patent Literature 2), and paperboard has been proposed. A method of introducing the curtain coating method to coated paper for general printing has also been proposed. For example, in order to solve a problem of craters from a coating color surface, a method has been proposed in which a suitable thickening agent is added to a coating liquid to provide a property (spinnability) with which the coating liquid is less likely to be cut even when the coating liquid is elongated (Patent Literature 3).

However, in the curtain coating method, unless the solid content, viscosity, spinnability, and the like of the coating liquid are controlled in appropriate ranges, the stability of the curtain film decreases when the coating liquid is continuously applied for a long time, resulting in an operational problem such as an occurrence of film breakage. Furthermore, addition of a thickening agent tends to decrease the stability of the coating liquid, for example, the viscosity of

the coating liquid increases with time, resulting in the deterioration of a liquid feed property and handleability.

In the curtain coating method, unless the static surface tension and the like of the coating liquid is controlled in appropriate ranges, "neck-in" occurs in which unevenness of the film thickness is generated at a central portion and end portions in the width direction of a base material due to an attempt to reduce the width of the curtain film by the surface tension of the coating liquid.

#### CITATION LIST

##### Patent Literature

PTL 1: Japanese Unexamined Patent Application Publication No. 54-085811

PTL 2: Japanese Unexamined Patent Application Publication No. 54-074761

PTL 3: Japanese Unexamined Patent Application Publication No. 06-294099

#### SUMMARY OF INVENTION

##### Technical Problem

An object of the present invention is to provide a method for manufacturing a paper barrier base material, in which good stability of a coating liquid and good continuous operability are achieved.

##### Solution to Problem

The solution to problem in the present invention is as follows.

1. A method for manufacturing a paper barrier base material, including a step of applying a water vapor barrier layer coating liquid that contains at least a water vapor barrier resin and a pigment onto a paper base material by a curtain coating method to form a water vapor barrier layer, in which the water vapor barrier layer coating liquid has

a spinnability of 0.07 seconds or more and 0.4 seconds or less at a solid content concentration of 32% by weight and a temperature of 25° C.

2. The method for manufacturing a paper barrier base material according to 1., in which the water vapor barrier layer coating liquid contains a viscosity modifier.

3. The method for manufacturing a paper barrier base material according to 2., in which the viscosity modifier contains ethylene-modified polyvinyl alcohol.

4. The method for manufacturing a paper barrier base material according to 3., in which a blending quantity of the ethylene-modified polyvinyl alcohol is 1% by weight or more and 20% by weight or less in terms of solid content relative to the pigment in the water vapor barrier layer coating liquid.

5. The method for manufacturing a paper barrier base material according to 2., in which the viscosity modifier contains sodium polyacrylate.

6. The method for manufacturing a paper barrier base material according to 5., in which a blending quantity of the sodium polyacrylate is 0.01% by weight or more and 0.5% by weight or less in terms of solid content relative to the pigment in the water vapor barrier layer coating liquid.

7. The method for manufacturing a paper barrier base material according to any one of 1. to 6., in which the water vapor barrier layer coating liquid further contains a water repellent and a surface-active agent and has a static surface

tension of 40 mN/m or less at a solid content concentration of 32% by weight and a temperature of 25° C.

8. The method for manufacturing a paper barrier base material according to 7., in which the water repellent contains a paraffin water repellent.

9. The method for manufacturing a paper barrier base material according to 7. or 8., in which a blending quantity of the water repellent is 20 parts by weight or more and 100 parts by weight or less in terms of solid content relative to 100 parts by weight of the pigment in the water vapor barrier layer coating liquid.

10. The method for manufacturing a paper barrier base material according to any one of 7. to 9., in which a blending quantity of the surface-active agent is 0.3 parts by weight or more and 3.0 parts by weight or less in terms of solid content relative to 100 parts by weight of the pigment in the water vapor barrier layer coating liquid.

11. The method for manufacturing a paper barrier base material according to any one of 1. to 10., in which the water vapor barrier layer coating liquid has a solid content concentration of 25% by weight or more and 45% by weight or less.

12. The method for manufacturing a paper barrier base material according to any one of 1. to 11., including a step of applying a gas barrier layer coating liquid onto the water vapor barrier layer to form a gas barrier layer.

##### Advantageous Effects of Invention

30 In the manufacturing method according to the present invention, a coating liquid has good stability, and it is possible to suppress an operational problem, such as film breakage, caused by continuous coating for a long time by the curtain coating method. Furthermore, by controlling the static surface tension, the occurrence of neck-in is suppressed, and coating can be performed without unevenness of the layer thickness in the width direction.

#### DESCRIPTION OF EMBODIMENTS

The present invention relates to a method for manufacturing a paper barrier base material, the method including: a step of applying a water vapor barrier layer coating liquid that contains at least a water vapor barrier resin and a pigment onto a paper base material by a curtain coating method to form a water vapor barrier layer, in which the water vapor barrier layer coating liquid has a spinnability of 0.07 seconds or more and 0.4 seconds or less at a solid content concentration of 32% by weight and a temperature of 25° C.

##### "Method for Manufacturing Paper Barrier Base Material"

A paper barrier base material is manufactured by applying a water vapor barrier layer coating liquid that contains at least a water vapor barrier resin and a pigment onto a paper base material by a curtain coating method to form a water vapor barrier layer.

The curtain coating method is a coating method in which a coating liquid is allowed to flow down in a curtain shape to form a curtain film, and a base material is passed through the curtain film to thereby provide a coating layer on the base material. The curtain coating method is contour coating in which a coating layer is formed along a base material and is a so-called pre-metered method as described above. Thus, the curtain coating method has a feature that the coating quantity is easily controlled.

In the present invention, when the water vapor barrier layer coating liquid is applied by a curtain coating method,

a known machine used in the curtain coating method can be used. It is possible to use any coating machine such as a slot-type curtain coating machine in which a curtain film is directly formed by discharging a coating liquid downward from a die, and a slide-type curtain coating machine in which a curtain film is formed by discharging a coating liquid upward from a die, allowing the coating liquid to flow while forming a film of the coating liquid on an inclined surface of the die, and then allowing the coating liquid to leave from the die and to freely fall.

(Water Vapor Barrier Layer Coating Liquid)

The water vapor barrier layer coating liquid is a coating liquid that contains at least a water vapor barrier resin and a pigment and that is primarily composed of water in which the water vapor barrier resin and the pigment are dissolved and dispersed and is characterized by having a spinnability of 0.07 seconds or more and 0.4 seconds or less at a solid content concentration of 32% by weight and a temperature of 25° C. The water vapor barrier layer coating liquid in the present invention contains at least a water vapor barrier resin and a pigment and may contain, for example, a water-soluble polymer, a crosslinking agent, a water repellent, and a viscosity modifier described in detail below.

Herein, the spinnability of a coating liquid is an index of the ease of extension of the coating liquid and is a value measured by an extensional viscometer. Specifically, the spinnability is determined by: 1) using a viscometer that includes a pair of circular plates having a diameter of 8 mm and arranged coaxially such that the axis is perpendicular, and enclosing a coating liquid having a liquid temperature of 25° C. between the plates (gap: 1 mm), 2) pulling up the upper plate perpendicularly by 8 mm at a speed of 400 mm/sec and holding the plate as it is, and 3) measuring the time from the start of pulling up of the plate to the occurrence of breakage of a coating liquid filament. The time until the filament is broken is preferably measured by a laser, and the time resolution at this time is preferably about 2 ms. Examples of the extensional viscometer capable of performing such measurement include an extensional viscometer (model name: CaBER 1) manufactured by Thermo Haake Inc.

In the curtain coating method, at the moment when a curtain film comes into contact with a base material, the curtain film is pulled by the base material and extended due to the difference between a falling speed of the curtain film and a traveling speed of the base material. When the spinnability of the coating liquid is 0.07 seconds or more, the curtain film can follow this extension, and a stable curtain film can be formed. If the spinnability is shorter than 0.07 seconds, the curtain film cannot follow this extension. Accordingly, the stability of the curtain film decreases, resulting in the occurrence of an operational problem such as occurrence of film breakage. On the other hand, if the spinnability exceeds 0.4 seconds, the curtain film excessively follows the base material and shakes in the flowing direction of the base material, also resulting in the occurrence of an operational problem such as film breakage. The spinnability of the water vapor barrier layer coating liquid at a solid content concentration of 32% by weight and a temperature of 25° C. is preferably 0.3 seconds or less.

The water vapor barrier layer coating liquid used in the preset invention preferably has a B-type viscosity in a range of 100 mPa·s or more and 1,500 mPa·s or less at a solid content concentration of 32% by weight and a temperature of 25° C. If the B-type viscosity is lower than 100 mPa·s, the coating liquid may excessively penetrate into the base material, and the quality of the resulting paper barrier base

material may be degraded. If the B-type viscosity is higher than 1,500 mPa·s, operational problems such as a poor liquid feed property and poor handleability of the coating liquid are likely to occur. The B-type viscosity of the coating liquid is a value measured with a Brookfield viscometer (B-type viscometer) using a No. 3 rotor at a rotation speed of 60 rpm.

The water vapor barrier layer coating liquid used in the preset invention preferably has a static surface tension of 40 mN/m or less at a solid content concentration of 32% by weight and a temperature of 25° C. When the static surface tension is 40 mN/m or less, the stability of a curtain film flowing down from a die increases, and even at a low flow rate, neck-in (a phenomenon in which unevenness of the film thickness is generated at a central portion and end portions due to shrinkage of the curtain film) of the curtain film and film breakage can be suppressed to facilitate the formation of a uniform and stable curtain film. The static surface tension at a solid content concentration of 32% by weight and a temperature of 25° C. is preferably 25 mN/m or more. If the static surface tension is less than 25 mN/m, the water vapor barrier layer coating liquid excessively penetrates into the base material due to excessive wettability of the water vapor barrier layer coating liquid to the base material, which may result in deterioration of the water vapor barrier property. The static surface tension of the coating liquid is a value measured by the plate method (Wilhelmy method) at a liquid temperature of 25° C. An example of a surface tensiometer capable of performing such measurement is a fully automatic surface tensiometer (model name: CBVP-Z) manufactured by Kyowa Interface Science Co., Ltd.

The properties such as the spinnability and static surface tension of the water vapor barrier layer coating liquid used in the present invention can be adjusted by, for example, the addition amounts of a viscosity modifier, a water repellent, a surface-active agent, and the like described in detail below and the blending ratio of the water vapor barrier resin, the pigment, and the like contained in the coating liquid. This is based on the magnitude of interaction between pigment particles and other compounds in the water vapor barrier layer coating liquid.

The solid content concentration of the water vapor barrier layer coating liquid used in the present invention is not particularly limited, but is preferably 25% by weight or more and more preferably 30% by weight or more. The upper limit of the solid content concentration is also not particularly limited, but is preferably 45% by weight or less and more preferably 40% by weight or less in consideration of, for example, a liquid feed property.

(Water Vapor Barrier Resin)

The water vapor barrier resin may be, for example, a synthetic adhesive such as a styrene-butadiene, styrene-acrylic, ethylene-vinyl acetate, paraffin (WAX), butadiene-methyl methacrylate, or vinyl acetate-butyl acrylate copolymer, a maleic anhydride copolymer, or an acrylic acid-methyl methacrylate copolymer; or a paraffin (WAX)-blended synthetic adhesive thereof. These may be used alone or as a mixture of two or more thereof. Of these, styrene-butadiene synthetic adhesives and styrene-acrylic synthetic adhesives are preferably used in view of the water vapor barrier property.

In the present invention, the styrene-butadiene synthetic adhesives refer to adhesives obtained by subjecting styrene and butadiene serving as main constituent monomers to emulsion polymerization in combination with various comonomers for modification. Examples of the comonomer include methyl methacrylate, acrylonitrile, acrylamide, hydroxyethyl acrylate, and unsaturated carboxylic acids

such as itaconic acid, maleic acid, and acrylic acid. As the emulsifier, an anionic surface-active agent such as sodium oleate, rosin acid soap, a sodium alkyl allyl sulfonate, or sodium dialkylsulfosuccinate may be used alone or in combination with a nonionic surface-active agent. An amphoteric or cationic surface-active agent may also be used depending on the purpose. The styrene-acrylic synthetic adhesives refer to adhesives obtained by subjecting styrene and acryl serving as main constituent monomers to emulsion polymerization in combination with various comonomers for modification.

(Water-Soluble Polymer)

Water-soluble polymers such as polyvinyl alcohols, e.g., fully saponified polyvinyl alcohol, partially saponified polyvinyl alcohol, and ethylene-copolymerized polyvinyl alcohol; proteins, e.g., casein, soybean protein, and synthetic proteins; starches, e.g., oxidized starch, cationic starch, urea phosphate esterified starch, and hydroxyethyl etherified starch; cellulose derivatives, e.g., carboxymethyl cellulose, hydroxymethyl cellulose, and hydroxyethyl cellulose; polyvinylpyrrolidone; and sodium alginate may be used in combination with the water vapor barrier resin as long as there is substantially no problem in the water vapor barrier property.

(Pigment)

The pigment increases the water vapor barrier property of the water vapor barrier layer and can improve the adhesion between the water vapor barrier layer and the gas barrier layer when the gas barrier layer is formed on the water vapor barrier layer by coating.

The pigment may be, for example, an inorganic pigment such as kaolin, clay, engineered kaolin, delaminated clay, ground calcium carbonate, precipitated calcium carbonate, mica, talc, titanium dioxide, barium sulfate, calcium sulfate, zinc oxide, silicic acid, a silicate, colloidal silica, or satin white; or a solid, hollow, or core-shell type organic pigment. These pigments may be used alone or as a mixture of two or more thereof.

Of these pigments, inorganic pigments such as kaolin, mica, and talc, which have a flat shape, are preferable, and kaolin and mica are more preferable from the viewpoints of both improving the water vapor barrier property and reducing the penetration of the gas barrier layer coating liquid. Of these, inorganic pigments having an aspect ratio of 10 or more are preferably used alone or as a mixture of two or more thereof. The aspect ratio is more preferably 100 or more and still more preferably 200 or more. In addition, inorganic pigments having a 50% volume-average particle size (D50) (hereinafter also referred to as an "average particle size") of 5  $\mu\text{m}$  or more are preferably used alone or as a mixture of two or more thereof. If the average particle size or the aspect ratio of the inorganic pigment used is smaller than the above range, the effect of improving the water vapor barrier property is reduced.

In the present invention, a pigment having an average particle size of 5  $\mu\text{m}$  or less may be further contained in the water vapor barrier layer that contains an inorganic pigment having an average particle size of 5  $\mu\text{m}$  or more to improve the water vapor barrier property and to improve the adhesion to the gas barrier layer. By using the pigment having an average particle size of 5  $\mu\text{m}$  or less in combination, voids in the water vapor barrier layer, the voids being formed by the inorganic pigment having an average particle size of 5  $\mu\text{m}$  or more, can be reduced. Thus, a better water vapor barrier property is exhibited. Specifically, in a case where a pigment having a different average particle size is contained in the water vapor barrier layer, the pigment having a small

average particle size fills voids formed by an inorganic pigment having a large average particle size in the water vapor barrier layer, and water vapor bypasses the pigment to pass through the water vapor barrier layer. Thus, it is surmised that the water vapor barrier layer has a higher water vapor barrier property than a water vapor barrier layer that does not contain such a pigment having a different average particle size.

In the present invention, in a case where an inorganic pigment having an average particle size of 5  $\mu\text{m}$  or more and a pigment having an average particle size of 5  $\mu\text{m}$  or less are used in combination, a blending ratio of the inorganic pigment having an average particle size of 5  $\mu\text{m}$  or more to the pigment having an average particle size of 5  $\mu\text{m}$  or less is preferably 50/50 to 99/1 on a dry weight basis. If the blending ratio of the inorganic pigment having an average particle size of 5  $\mu\text{m}$  or more is smaller than the above range, the number of times water vapor bypasses the water vapor barrier layer is reduced and the distance of the movement is shortened. Consequently, the effect of improving the water vapor barrier property may be reduced. On the other hand, if the blending ratio of the inorganic pigment having an average particle size of 5  $\mu\text{m}$  or more is larger than the above range, the voids formed by the inorganic pigment having a large average particle size in the water vapor barrier layer cannot be sufficiently filled with the pigment having an average particle size of 5  $\mu\text{m}$  or less. Therefore, a further improvement in the water vapor barrier property is not achieved.

In the present invention, the pigment having an average particle size of 5  $\mu\text{m}$  or less and used in combination with the inorganic pigment having an average particle size of 5  $\mu\text{m}$  or more may be, for example, an inorganic pigment such as kaolin, clay, engineered kaolin, delaminated clay, ground calcium carbonate, precipitated calcium carbonate, talc, titanium dioxide, barium sulfate, calcium sulfate, zinc oxide, silicic acid, a silicate, colloidal silica, or satin white; or a solid, hollow, or core-shell type organic pigment. These pigments may be used alone or as a mixture of two or more thereof. Of these pigments, ground calcium carbonate is preferably used.

When a pigment is contained in the water vapor barrier layer, the blending quantity of the total of the water vapor barrier resin and the water-soluble polymer relative to the pigment is, in terms of solid content, preferably in a range of 5 parts by weight or more and 200 parts by weight or less, and more preferably 10 parts by weight or more and 150 parts by weight or less relative to 100 parts by weight of the pigment.

(Crosslinking Agent)

In the present invention, a crosslinking agent typified by a polyvalent metal salt or the like may be added to the water vapor barrier layer. Since the crosslinking agent causes a crosslinking reaction with a water vapor barrier resin or water-soluble polymer contained in the water vapor barrier layer, the number of bonds (crosslinked points) in the water vapor barrier layer increases. That is, the water vapor barrier layer has a dense structure and can exhibit a good water vapor barrier property.

In the present invention, the type of crosslinking agent is not particularly limited, and it is possible to appropriately select and use a polyvalent metal salt (compound in which a polyvalent metal such as copper, zinc, silver, iron, potassium, sodium, zirconium, aluminum, calcium, barium, magnesium, or titanium is bound to an ionic substance such as a carbonate ion, a sulfate ion, a nitrate ion, a phosphate ion, a silicate ion, a nitrogen oxide, or a boron oxide), an amine

compound, an amide compound, an aldehyde compound, a hydroxy acid, or the like in accordance with the types of the water vapor barrier resin and water-soluble polymer contained in the water vapor barrier layer.

In a case of using a styrene water vapor barrier resin such as a styrene-butadiene or a styrene-acrylic resin, which exhibits a good effect in the water-vapor barrier property, a polyvalent metal salt is preferably used, and potassium alum is more preferably used from the viewpoint of exhibiting the crosslinking effect. The blending quantity of the crosslinking agent is not particularly limited within a range of a coatable coating liquid concentration or coating liquid viscosity. The blending quantity of the crosslinking agent is preferably 1 part by weight or more and 10 parts by weight or less and more preferably 3 parts by weight or more and 5 parts by weight or less relative to 100 parts by weight of the pigment. If the blending quantity is less than 1 part by weight, the effect of adding the crosslinking agent may not be sufficiently achieved. If the blending quantity is more than 10 parts by weight, the viscosity of the coating liquid may significantly increase, resulting in a difficulty of coating.

In the present invention, in a case where the crosslinking agent is added to the water vapor barrier layer coating liquid, it is preferable that the crosslinking agent be dissolved in a polar solvent such as ammonia and then added to the coating liquid. When the crosslinking agent is dissolved in the polar solvent, a bond is formed between the crosslinking agent and the polar solvent. Therefore, a crosslinking reaction with the water vapor barrier resin or the water-soluble polymer does not occur immediately after the addition of the crosslinking agent to the coating liquid. Thus, an increase in the viscosity of the coating liquid can be suppressed. It is supposed that, in such a case, the polar solvent component is volatilized by drying after coating on the paper base material, a crosslinking reaction with the water vapor barrier resin or the water-soluble polymer occurs, and a dense water vapor barrier layer is formed.

#### (Water Repellent)

In the present invention, from the viewpoint of improving the water vapor barrier property, a water repellent is preferably contained in the water vapor barrier layer. Examples of the water repellent include paraffin water repellents primarily constituted by alkane compounds; natural oil water repellents derived from animal or plant, such as carnauba and lanolin; silicone-containing water repellents that contain silicone or a silicone compound; and fluorine-containing water repellents that contain a fluorine compound. Of these, paraffin water repellents are preferably used from the viewpoint of exhibiting the water vapor barrier performance. These water repellents may be used alone or as a mixture of two or more thereof.

In the present invention, the blending quantity of the water repellent is not particularly limited, but the blending quantity of the water repellent is, in terms of solid content, preferably 1 part by weight or more and 100 parts by weight or less relative to 100 parts by weight of the total of the water vapor barrier resin and the water-soluble polymer. If the blending quantity of the water repellent is less than 1 part by weight, the effect of improving the water vapor barrier property may not be sufficiently achieved. On the other hand, if the blending quantity of the water repellent exceeds 100 parts by weight, in a case where a gas barrier layer is provided on the water vapor barrier layer, it becomes difficult to uniformly form the gas barrier layer, which may result in deterioration of the gas barrier property.

#### (Surface-Active Agent)

In the present invention, from the viewpoint of an improvement in the leveling property of the water vapor barrier layer coating liquid and the adhesion to the gas barrier layer, a surface-active agent is preferably contained in the water vapor barrier layer. The ionic property of the surface-active agent is not limited, and any type of surface-active agent such as an anionic surface-active agent, a cationic surface-active agent, an amphoteric surface-active agent, or a nonionic surface-active agent may be used. These surface-active agents may be used alone or in combination of two or more thereof. Examples of the specific type of surface-active agent include silicone surface-active agents, fluorine surface-active agents, alcohol surface-active agents, acetylene surface-active agents having an acetylene group, acetylene diol surface-active agents having an acetylene group and two hydroxyl groups, alkyl sulfonate surface-active agents having an alkyl group and a sulfonic acid, ester surface-active agents, amide surface-active agents, amine surface-active agents, alkyl ether surface-active agents, phenyl ether surface-active agents, sulfate ester surface-active agents, and phenol surface-active agents. Of these, acetylene diol surface-active agents, which exhibit a high effect of improving the leveling property of the water vapor barrier layer coating liquid, are preferably used. The improvement in the leveling property of the water vapor barrier layer coating liquid improves the uniformity of the resulting water vapor barrier layer and facilitates the formation of a uniform gas barrier layer when the gas barrier layer is provided on the water vapor barrier layer. Consequently, the adhesion between the water vapor barrier layer and the gas barrier layer is improved, and both the water vapor barrier property and the gas barrier property tend to be improved.

In the present invention, the blending quantity of the surface-active agent is not particularly limited, but the blending quantity of the surface-active agent is, in terms of solid content, preferably 0.3 parts by weight or more and 3.0 parts by weight or less, and more preferably 0.3 parts by weight or more and 2.0 parts by weight or less relative to 100 parts by weight of the pigment in the water vapor barrier layer. If the blending quantity of the surface-active agent is less than 0.3 parts by weight, the effect of improving the leveling property of the water vapor barrier layer coating liquid may not be sufficiently achieved. On the other hand, if the blending quantity of the surface-active agent exceeds 3.0 parts by weight, the effect of improving the leveling property of the water vapor barrier layer coating liquid may be saturated, and the water vapor barrier property may be deteriorated.

#### (Viscosity Modifier)

In the present invention, the water vapor barrier layer coating liquid preferably contains a viscosity modifier. The viscosity modifier is a chemical agent having an action of adjusting the flowability of the coating liquid. Containing the viscosity modifier makes it easy to control the spinnability of the water vapor barrier layer coating liquid to a desired value.

Specific examples of the viscosity modifier include hydrophilic polymers such as polyvinylpyrrolidone resins, polyvinyl alcohol resins, cellulose resins, polyacrylamide resins, and poly(meth)acrylic acid resins. Of these, ethylene-modified polyvinyl alcohol and sodium polyacrylate are preferred because the degree of deterioration of the water vapor barrier property due to the addition of the viscosity modifier is low and coating suitability by the curtain coating method is good. In particular, ethylene-modified polyvinyl alcohol is preferable because ethylene-modified polyvinyl alcohol is a

## 11

hydrophobic group-introduced polymer and thus has less influence on the water vapor barrier property despite being a hydrophilic polymer.

Since the viscosity modifier is hydrophilic, a large amount of viscosity modifier added may deteriorate the water vapor barrier property. In addition, since the stability and continuous operability of the coating liquid also tend to decrease, the amount of viscosity modifier added is preferably small as long as the spinnability of the water vapor barrier layer coating liquid can be 0.07 seconds or more. For example, the amount of ethylene-modified polyvinyl alcohol added is preferably 1% by weight or more and 20% by weight or less, and more preferably 1% by weight or more and 10% by weight or less in terms of solid content relative to the pigment in the water vapor barrier layer coating liquid. The amount of sodium polyacrylate added is preferably 0.01% by weight or more and 0.5% by weight or less, and more preferably 0.01% by weight or more and 0.1% by weight or less in terms of solid content relative to the pigment in the water vapor barrier layer coating liquid.

In the water vapor barrier layer coating liquid, in addition to the water vapor barrier resin, the water-soluble polymer, the pigment, the crosslinking agent, the water repellent, the surface-active agent, and the viscosity modifier described above, various commonly used auxiliary agents such as a dispersant, an antifoaming agent, a water-resistant agent, a dye, and a fluorescent dye may be used.

In the present invention, the coating quantity of the water vapor barrier layer is preferably 3 g/m<sup>2</sup> or more and 50 g/m<sup>2</sup> or less, more preferably 5 g/m<sup>2</sup> or more and 40 g/m<sup>2</sup> or less, and still more preferably 7 g/m<sup>2</sup> or more and 30 g/m<sup>2</sup> or less on a dry weight basis. If the coating quantity of the water vapor barrier layer is less than 3 g/m<sup>2</sup>, it becomes difficult to completely cover the paper base material with the coating liquid, and thus a sufficient water vapor barrier property may not be achieved or when the gas barrier layer coating liquid is applied onto the water vapor barrier layer, the gas barrier layer coating liquid may penetrate into the paper base material, and thus a sufficient gas barrier property may not be achieved. On the other hand, if the coating quantity of the water vapor barrier layer is larger than 50 g/m<sup>2</sup>, the drying load in coating increases.

It should be noted that, in the present invention, the water vapor barrier layer may be formed of a single layer or may have a multilayer structure including two or more layers. In a case where the water vapor barrier layer has a multilayer structure including two or more layers, the total coating quantity of all the water vapor barrier layers is preferably within the above range.

## (Paper Base Material)

In the present invention, the paper base material is a sheet composed of pulp, a filler, various auxiliary agents, and the like.

The pulp used may be, for example, chemical pulp such as hardwood bleached kraft pulp (LBKP), softwood bleached kraft pulp (NBKP), hardwood unbleached kraft pulp (LUKP), softwood unbleached kraft pulp (NUKP), or sulfite pulp; mechanical pulp such as stone groundwood pulp or thermo-mechanical pulp; wood fibers such as de-inked pulp or recycled paper pulp; or non-wood fibers derived from kenaf, bamboo, hemp, or the like. The pulp may be used in combination as appropriate. Of these, chemical pulp or mechanical pulp is preferably used, and chemical pulp is more preferably used because, for example, foreign matter is unlikely to be mixed into the base paper, discoloration over time is unlikely to occur when used paper containers are supplied as a used paper raw material and

## 12

used for recycling, and good surface texture is obtained when printed because the above pulp has a high degree of whiteness, and consequently, high value is added particularly when the pulp is used as a packaging material.

5 The filler used may be known filler such as white carbon, talc, kaolin, clay, ground calcium carbonate, precipitated calcium carbonate, titanium oxide, zeolite, or synthetic resin filler. In addition, internal auxiliary agents for papermaking, such as aluminum sulfate or any of various anionic, cationic, 10 nonionic, or amphoteric retention aids, drainage aids, paper strengthening agents, and internal sizing agents may be used, as necessary. Furthermore, for example, dyes, fluorescent whitening agents, pH adjusting agents, antifoaming agents, pitch control agents, and slime control agents may 15 also be added, as necessary.

The method for manufacturing a paper base material (papermaking) is not particularly limited. The paper base material can be manufactured according to the acidic papermaking, neutral papermaking, or alkaline papermaking 20 method using any known machine such as a Fourdrinier former, on-top hybrid former, or gap former machine. The paper base material may be formed of a single layer or may have a multilayer structure including two or more layers.

Furthermore, the surface of the paper base material can be 25 treated with various chemical agents. Examples of chemical agents that may be used include oxidized starch, hydroxyethyl etherified starch, enzyme-modified starch, polyacrylamide, polyvinyl alcohol, surface sizing agents, water-resistant agents, water-retention agents, thickening agents, and 30 lubricants. These chemical agents may be used alone or as a mixture of two or more thereof. Furthermore, these various chemical agents may be used in combination with pigments. The pigment may be, for example, an inorganic pigment such as kaolin, clay, engineered kaolin, delaminated clay, 35 ground calcium carbonate, precipitated calcium carbonate, mica, talc, titanium dioxide, barium sulfate, calcium sulfate, zinc oxide, silicic acid, a silicate, colloidal silica, or satin white; or a solid, hollow, or core-shell type organic pigment. These pigments may be used alone or as a mixture of two or 40 more thereof.

The method for treating the surface of the paper base material is not particularly limited. Any known coating machine such as a rod-metering size press, a pond size press, a gate-roll coater, a spray coater, a blade coater, or a curtain 45 coater may be used.

Examples of the paper base material obtained in this manner include various known paper base materials such as high-quality paper, medium quality paper, coated paper, one side glossy paper, kraft paper, one side glossy kraft paper, 50 bleached kraft paper, glassine paper, paperboard, white paperboard, and liner.

The grammage of the paper base material can be appropriately selected in accordance with, for example, various qualities desired for the paper barrier base material and 55 handleability but is usually preferably about 20 g/m<sup>2</sup> or more and about 500 g/m<sup>2</sup> or less. In a case of a paper barrier packaging material used for packaging applications such as packaging materials, containers, and cups for food and the like, a paper barrier packaging material having a grammage of 25 g/m<sup>2</sup> or more and 400 g/m<sup>2</sup> or less is more preferable. In particular, in a case of a paper barrier packaging material used for soft packaging materials described later, a paper barrier packaging material having a grammage of 30 g/m<sup>2</sup> or more and 110 g/m<sup>2</sup> or less is more preferable.

## 60 (Gas Barrier Layer)

The method for manufacturing a paper barrier base material according to the present invention may include applying

a gas barrier layer coating liquid onto the water vapor barrier layer to form a gas barrier layer. The gas barrier layer coating liquid is preferably a coating liquid that is primarily composed of water in which polymers such as a water-soluble polymer and a water-dispersible polymer are dissolved and dispersed. The paper barrier base material according to the present invention including a gas barrier layer that contains polymers such as a water-soluble polymer and a water-dispersible polymer has a good water vapor barrier property and a good gas barrier property.

Examples of the water-soluble polymer used for the gas barrier layer in the present invention include polyvinyl alcohols such as fully saponified polyvinyl alcohol, partially saponified polyvinyl alcohol, and ethylene-copolymerized polyvinyl alcohol; proteins such as casein, soybean protein, and synthetic proteins; starches such as oxidized starch, cationic starch, urea phosphate esterified starch, and hydroxyethyl etherified starch; cellulose derivatives such as carboxymethyl cellulose, hydroxymethyl cellulose, and hydroxyethyl cellulose; polyvinylpyrrolidone; and sodium alginate. Of these, polyvinyl alcohols and cellulose derivatives are preferable, and polyvinyl alcohols are more preferable from the viewpoint of the gas barrier property.

Examples of the water-dispersible polymer used for the gas barrier layer include polyvinylidene chloride, ethylene vinyl acetate resins, and modified polyolefin resins.

In the present invention, containing a pigment in the gas barrier layer is preferable from the viewpoint of improving the gas barrier property. The pigment used in the gas barrier layer may be, for example, an inorganic pigment such as kaolin, clay, engineered kaolin, delaminated clay, ground calcium carbonate, precipitated calcium carbonate, mica, talc, titanium dioxide, barium sulfate, calcium sulfate, zinc oxide, silicic acid, a silicate, colloidal silica, or satin white; or a solid, hollow, or core-shell type organic pigment. These pigments may be used alone or as a mixture of two or more thereof.

Of these pigments, inorganic pigments such as kaolin, mica, and talc, which have a flat shape, are preferable, and kaolin and mica are more preferable from the viewpoint of improving the gas barrier property. An inorganic pigment having an average particle size of 3  $\mu\text{m}$  or more is more preferably used, and an inorganic pigment having an average particle size of 5  $\mu\text{m}$  or more is still more preferably used. An inorganic pigment having an aspect ratio of 10 or more is more preferably used, and an inorganic pigment having an aspect ratio of 30 or more is still more preferably used.

In a case where a pigment is contained in the gas barrier layer, a gas such as oxygen bypasses the pigment to pass through the gas barrier layer. Therefore, the gas barrier layer has a better gas barrier property under a high-humidity atmosphere than a gas barrier layer composed of a polymer such as a water-soluble polymer and/or a water-dispersible polymer that does not contain a pigment.

In the present invention, when a pigment is contained in the gas barrier layer, the blending ratio of the pigment to the water-soluble polymer and the water-dispersible polymer is preferably pigment/(total of water-soluble polymer and water-dispersible polymer)=1/100 to 1000/100 on a dry weight basis. If the ratio of the pigment is out of the above range, the effect of improving the gas barrier property may be reduced.

It should be noted that, in the present invention, in blending the pigment in the water-soluble polymer and the water-dispersible polymer, the pigment is preferably added to and mixed with the polymers in the form of a slurry.

In the present invention, a crosslinking agent typified by a polyvalent metal salt or the like may be added to the gas barrier layer. Since the crosslinking agent causes a crosslinking reaction with a polymer such as a water-soluble polymer or water-dispersible polymer contained in the gas barrier layer, the number of bonds (crosslinked points) in the gas barrier layer increases. That is, the gas barrier layer has a dense structure and can exhibit a good gas barrier property.

In the present invention, the type of crosslinking agent is not particularly limited, and it is possible to appropriately select and use a polyvalent metal salt (compound in which a polyvalent metal such as copper, zinc, silver, iron, potassium, sodium, zirconium, aluminum, calcium, barium, magnesium, or titanium is bound to an ionic substance such as a carbonate ion, a sulfate ion, a nitrate ion, a phosphate ion, a silicate ion, a nitrogen oxide, or a boron oxide), an amine compound, an amide compound, an aldehyde compound, a hydroxy acid, or the like in accordance with the type of polymer such as the water-soluble polymer or water-dispersible polymer contained in the gas barrier layer. From the viewpoint of exhibiting the crosslinking effect, a polyvalent metal salt is preferably used, and potassium alum is more preferably used.

The blending quantity of the crosslinking agent is not particularly limited within a range of a coatable coating liquid concentration or coating liquid viscosity. The blending quantity of the crosslinking agent is preferably 1 part by weight or more and 10 parts by weight or less and more preferably 3 parts by weight or more and 5 parts by weight or less relative to 100 parts by weight of the pigment. If the blending quantity is less than 1 part by weight, the effect of adding the crosslinking agent may not be sufficiently achieved. If the blending quantity is more than 10 parts by weight, the viscosity of the coating liquid may significantly increase, resulting in a difficulty of coating.

(Surface-Active Agent)

In the present invention, a surface-active agent is preferably contained in the gas barrier layer from the viewpoint of adhesion to the water vapor barrier layer. The ionic property of the surface-active agent is not limited, and any type of surface-active agent such as an anionic surface-active agent, a cationic surface-active agent, an amphoteric surface-active agent, or a nonionic surface-active agent may be used. These surface-active agents may be used alone or in combination of two or more thereof. Examples of the specific type of surface-active agent include silicone surface-active agents, fluorine surface-active agents, alcohol surface-active agents, acetylene surface-active agents having an acetylene group, acetylene diol surface-active agents having an acetylene group and two hydroxyl groups, alkyl sulfonate surface-active agents having an alkyl group and a sulfonic acid, ester surface-active agents, amide surface-active agents, amine surface-active agents, alkyl ether surface-active agents, phenyl ether surface-active agents, sulfate ester surface-active agents, and phenol surface-active agents. Of these, acetylene diol surface-active agents, which exhibit a high effect of improving the leveling property of the coating liquid, are preferably used. The improvement in the leveling property of the coating liquid improves uniformity of the gas barrier layer, and thus the gas barrier property is improved.

In the gas barrier layer in the present invention, in addition to the water-soluble polymer and the pigment described above, various commonly used auxiliary agents such as a dispersant, a thickening agent, a water-retention agent, an antifoaming agent, a water-resistant agent, a dye, and a fluorescent dye may be used.

In the present invention, the coating quantity of the gas barrier layer is preferably 0.2 g/m<sup>2</sup> or more and 20 g/m<sup>2</sup> or less on a dry weight basis. If the coating quantity of the gas barrier layer is less than 0.2 g/m<sup>2</sup>, it is difficult to form a uniform gas barrier layer, and thus a sufficient gas barrier property may not be achieved. On the other hand, if the coating quantity of the gas barrier layer is larger than 20 g/m<sup>2</sup>, the drying load in coating increases.

It should be noted that, in the present invention, the gas barrier layer may be formed of a single layer or may have a multilayer structure including two or more layers. In a case where the gas barrier layer has a multilayer structure including two or more layers, the total coating quantity of all the gas barrier layers is preferably within the above range.

In a case of applying the gas barrier layer onto the water vapor barrier layer, the coating method of the gas barrier layer is not particularly limited. Examples of the method include methods using a curtain coater, a blade coater, a bar coater, a roll coater, an air knife coater, a reverse roll coater, a spray coater, a size press coater, or a gate roll coater. (Paper Barrier Base Material)

A paper barrier base material according to the present invention is manufactured by at least applying a water vapor barrier layer coating liquid onto a paper base material by a curtain coating method, and then performing a usual drying step. In a preferred embodiment, the paper barrier base material is finished such that the water content of the coated paper after manufacturing becomes about 3% by weight or more and about 10% by weight or less, more preferably about 4% by weight or more and about 8% by weight or less. As a method for drying the water vapor barrier layer and the gas barrier layer, for example, a usual method using a steam heater, a gas heater, an infrared heater, an electric heater, a hot air heater, microwaves, a cylinder drier, or the like is employed. For the smoothing process, a typical smoothing device such as a super calender, a gloss calender, a soft calender, a thermal calender, or a shoe calender can be used. The smoothing device is appropriately used on-machine or off-machine, and the form of a pressing device, the number of pressing nips, heating, and the like are also appropriately adjusted.

The paper barrier base material according to the present invention may be used without further treatment, or laminated with a resin or the like, or may be attached to a general-purpose film, a barrier film, aluminum foil, or the like to form a paper barrier packaging material used for packaging applications such as packaging materials, containers, and cups for food and the like, or a laminate used for, for example, industrial materials.

Of these, the paper barrier base material according to the present invention can be suitably used as a paper barrier packaging material used for packaging applications such as packaging materials, containers, and cups for food and the like and can be particularly suitably used as a soft packaging material for food and the like. It should be noted that the soft packaging material is, in terms of configuration, a packaging material formed of a material rich in flexibility, and generally refers to a packaging material formed of a thin and flexible material such as paper, a film, or aluminum foil alone or formed of such thin and flexible materials that are attached together. The soft packaging material refers to, in terms of shape, a packaging material, such as a bag, which maintains its three-dimensional shape when the contents are put therein.

When the paper barrier base material according to the present invention is used as a packaging material, in particular, a soft packaging material, for food and the like, the

paper barrier base material may be laminated with a resin having a heat sealing property. In such a case, it is possible to enhance the airtightness of the packaging material, to protect the contents from, for example, oxidation due to oxygen and deterioration due to moisture or the like, and to extend the preservation period.

When the paper barrier base material according to the present invention is used as a laminate used for an industrial material or the like, intrusion of oxygen and moisture can be suppressed to prevent decay and deterioration, and in addition, an effect such as a flavor barrier property to prevent the odor of a solvent from leaking out is also expected.

## EXAMPLES

The present invention will now be specifically described with reference to Examples; however, it goes without saying that the present invention is not limited to these examples.

It should be noted that, unless otherwise specified, "part" and "%" in the examples refer to "part by weight" and "% by weight", respectively. The obtained paper barrier base materials were tested in accordance with the evaluation methods described below.

### (Evaluation Method)

#### <Water Vapor Permeability (Water Vapor Barrier Property)>

The water vapor permeability was measured by using a moisture permeability measuring device (L80-4000, manufactured by Dr. Lyssy) in accordance with JIS K7129A: 2008 at a temperature of 40±0.5°C. and a relative humidity difference of 90±2%.

#### <Oxygen Permeability (Gas Barrier Property)>

The oxygen permeability was measured under the condition of 23°C.-0% RH by using OX-TRAN2/21 manufactured by MOCON Inc.

#### <Spinnability>

The spinnability of the obtained water vapor barrier layer coating liquid with a solid content concentration of 32% by weight at a temperature of 25°C. immediately after preparation was measured with an extensional viscometer (CaBER 1, manufactured by Thermo Haake Inc.).

#### <B-Type Viscosity>

The viscosity of the obtained water vapor barrier layer coating liquid with a solid content concentration of 32% by weight at a temperature of 25°C. immediately after preparation was measured with a Brookfield viscometer (BII viscometer, manufactured by Tokyo Keiki Inc.) using a No. 3 rotor at a rotation speed of 60 rpm.

#### <Static Surface Tension>

The static surface tension of the obtained water vapor barrier layer coating liquid with a solid content concentration of 32% by weight at a temperature of 25°C. immediately after preparation was measured with a fully automatic surface tensiometer (CBVP-Z, manufactured by Kyowa Interface Science Co., Ltd.).

#### <Stability of Coating Liquid>

For the obtained water vapor barrier layer coating liquid (solid content concentration: 32% by weight), a viscosity immediately after preparation and a viscosity after standing at a temperature of 25°C. for 12 hours were measured with a Brookfield viscometer (BII viscometer, manufactured by Tokyo Keiki Inc.) using a No. 3 rotor at a temperature of 25°C. and a rotation speed of 60 rpm.

On the basis of the difference in viscosity before and after standing, the stability of the coating liquid was evaluated in accordance with the following criteria.

## (Evaluation Criteria)

○: The difference in viscosity before and after standing is less than 500 mPa·s.

x: The difference in viscosity before and after standing is 500 mPa·s or more.

## &lt;Continuous Operability&gt;

The water vapor barrier layer coating liquid immediately after preparation was continuously applied on 18,000 m (for one hour) by using a curtain coater at a coating speed of 300 m/min such that the coating quantity was 10 g/m<sup>2</sup> on a dry weight basis, and the number of times that film breakage occurred in a curtain film was determined to evaluate continuous operability in accordance with the following criteria.

## (Evaluation Criteria)

○: The number of times that film breakage occurred was zero (film breakage did not occur).

Δ: The number of times that film breakage occurred was one.

x: The number of times that film breakage occurred was two or more.

## &lt;Neck-In&gt;

Under the conditions where a water vapor barrier layer coating liquid was supplied from a curtain head, and the falling height of the water vapor barrier layer coating liquid (the distance from the curtain head to a base material) was 100 mm, the neck-in was assumed to occur when the width of a curtain film, upon coming in contact with the base material, became 95% or less relative to the width of the curtain head, and the frequency of the occurrence of the neck-in was determined in accordance with the following criteria:

○: Neck-in occurred less than once within 10 minutes.

Δ: Neck-in occurred once or more within 10 minutes and less than once within one minute.

x: Neck-in occurred once or more within one minute.

## Example 1

## (Production of Paper Base Material)

Hardwood kraft pulp (LBKP) having a Canadian standard freeness (CSF) of 500 ml and softwood kraft pulp (NBKP) having a CSF of 530 ml were blended at a weight ratio of 80/20 to obtain material pulp.

To the material pulp, polyacrylamide (PAM) having a molecular weight of 2,500,000 was added as a dry paper strengthening agent in an amount of 0.1% per absolute dry pulp weight, an alkyl ketene dimer (AKD) was added as a sizing agent in an amount of 0.35% per absolute dry pulp weight, a polyamide epichlorohydrin (PAEH) resin was added as a wet paper strengthening agent in an amount of 0.15% per absolute dry pulp weight, and polyacrylamide (PAM) having a molecular weight of 10,000,000 was added as a retention aid in an amount of 0.08% per absolute dry pulp weight. Subsequently, the resulting mixture was put through a Fourdrinier papermaking machine to obtain paper with a grammage of 59 g/m<sup>2</sup>.

Next, polyvinyl alcohol (product name: PVA117, manufactured by Kuraray Co., Ltd.) that had been prepared to have a solid content concentration of 2% was applied to thus-obtained paper by using a rod-metering size press such that the total of the polyvinyl alcohol applied to both surfaces was 1.0 g/m<sup>2</sup> and then dried to obtain base paper with a grammage of 60 g/m<sup>2</sup>. The obtained base paper was smoothed by a single pass on a chilled calender at a speed of 300 min/m and a line pressure of 50 kgf/cm.

## (Preparation of Water Vapor Barrier Layer Coating Liquid A1)

To engineered kaolin (product name: Barrisurf HX, average particle size: 9.0 µm, aspect ratio: 80 to 100, manufactured by Imerys), polyacrylate soda was added (0.2% relative to the pigment) as a dispersant. The mixture was then dispersed in a Serie mixer to prepare a kaolin slurry having a solid content concentration of 60%. To 90 parts (solid content) of the kaolin slurry prepared above, 10 parts (solid content) of talc (product name: TALCRON, manufactured by Specialty MINERALS Inc.) was added to prepare a pigment slurry having a solid content concentration of 50%.

Into the pigment slurry prepared above, relative to 100 parts (solid content) of the pigment, 50 parts (solid content)

15 of a styrene-acrylic copolymer emulsion (product name: X-511-374E, manufactured by Sained Chemical Industry Co., Ltd.) and 50 parts (solid content) of an acrylic resin (product name: BARIASTAR ASN 1004, manufactured by Mitsui Chemicals, Inc.) were blended as water vapor barrier

20 resins. A viscosity modifier (ethylene-modified polyvinyl alcohol, product name: EXCEVAL RS4104, manufactured by Kuraray Co., Ltd.) was further blended such that the amount of the viscosity modifier was 5 parts (solid content). Thus, a water vapor barrier layer coating liquid A1 having a solid content concentration of 32% was obtained.

## (Preparation of Gas Barrier Layer Coating Liquid B1)

An aqueous solution of polyvinyl alcohol (product name: PVA117, manufactured by Kuraray Co., Ltd.) was prepared so as to have a solid content concentration of 12% to obtain 30 a gas barrier layer coating liquid B1. This gas barrier layer coating liquid B1 had a surface tension of 35 mN/m.

## (Production of Paper Barrier Base Material)

The water vapor barrier layer coating liquid A1 was applied to one surface of the obtained base paper with a curtain coater at a coating speed of 300 m/min such that the coating quantity was 10 g/m<sup>2</sup> on a dry weight basis, and dried. Subsequently, the gas barrier layer coating liquid B1 was applied to the water vapor barrier layer coating liquid A1 with a curtain coater at a coating speed of 300 m/min 35 such that the coating quantity was 5.0 g/m<sup>2</sup> on a dry weight basis. Thus, a paper barrier base material was obtained.

## Example 2

## 45 (Preparation of Water Vapor Barrier Layer Coating Liquid A2)

A water vapor barrier layer coating liquid A2 having a solid content concentration of 32% was obtained as in the water vapor barrier layer coating liquid A1 except that 5 parts (solid content) of the viscosity modifier (ethylene-modified polyvinyl alcohol) was changed to 0.05 parts (solid content) of a viscosity modifier (sodium polyacrylate, product name: ARONVIS MX, manufactured by TOAGOSEI Co., Ltd.).

55 A paper barrier base material was obtained as in Example 1 except that the water vapor barrier layer coating liquid A2 was used instead of the water vapor barrier layer coating liquid A1.

## Example 3

## 60 (Preparation of Water Vapor Barrier Layer Coating Liquid A3)

A water vapor barrier layer coating liquid A3 having a 65 solid content concentration of 32% was obtained as in the water vapor barrier layer coating liquid A1 except that 5 parts (solid content) of the viscosity modifier (ethylene-

19

modified polyvinyl alcohol) was changed to 0.3 parts (solid content) of a viscosity modifier (sodium polyacrylate, product name: ARONVIS MX, manufactured by TOAGOSEI Co., Ltd.).

A paper barrier base material was obtained as in Example 1 except that the water vapor barrier layer coating liquid A3 was used instead of the water vapor barrier layer coating liquid A1.

## Comparative Example 1

## (Preparation of Water Vapor Barrier Layer Coating Liquid A4)

A water vapor barrier layer coating liquid A4 having a solid content concentration of 32% was obtained as in the

20

## Example 4

## (Preparation of Water Vapor Barrier Layer Coating Liquid A6)

A water vapor barrier layer coating liquid A6 having a solid content concentration of 32% was obtained as in the water vapor barrier layer coating liquid A1 except that the blending quantity of the viscosity modifier (ethylene-modified polyvinyl alcohol) was changed to 15 parts (solid content).

A paper barrier base material was obtained as in Example 1 except that the water vapor barrier layer coating liquid A6 was used instead of the water vapor barrier layer coating liquid A1.

TABLE 1

|                                        |                                       | Example 1             | Example 2       | Example 3       | Example 4             | Comparative Example 1 | Comparative Example 2 |
|----------------------------------------|---------------------------------------|-----------------------|-----------------|-----------------|-----------------------|-----------------------|-----------------------|
| Coating liquid                         |                                       | A1                    | A2              | A3              | A6                    | A4                    | A5                    |
| Viscosity modifier                     |                                       | Ethylene-modified PVA | Na polyacrylate | Na polyacrylate | Ethylene-modified PVA | None                  | Na polyacrylate       |
| Quantity of viscosity modifier blended | parts by weight (relative to pigment) | 5.0                   | 0.05            | 0.3             | 15                    | —                     | 0.45                  |
| Coating color concentration            | %                                     | 32                    | 32              | 32              | 32                    | 32                    | 32                    |
| Spinnability                           | sec                                   | 0.08                  | 0.10            | 0.40            | 0.20                  | 0.03                  | 0.50                  |
| B-type viscosity                       | mPa · s                               | 300                   | 210             | 250             | 360                   | 200                   | 310                   |
| Static surface tension                 | mN/m                                  | 39                    | 39              | 39              | 38                    | 39                    | 39                    |
| Stability of coating liquid            |                                       | ○                     | ○               | ○               | ○                     | ○                     | X                     |
| Continuous operability                 |                                       | ○                     | ○               | △               | ○                     | X                     | X                     |
| Neck-in                                |                                       | ○                     | ○               | ○               | ○                     | ○                     | ○                     |
| Water vapor permeability               | g/m <sup>2</sup> · day                | 2.7                   | 2.9             | 3.0             | 2.8                   | 3.0                   | 3.3                   |
| Oxygen permeability                    | ml/m <sup>2</sup> · day               | 1.0                   | 1.0             | 1.0             | 1.0                   | 1.0                   | 1.0                   |

water vapor barrier layer coating liquid A1 except that no viscosity modifier was blended.

A paper barrier base material was obtained as in Example 1 except that the water vapor barrier layer coating liquid A4 was used instead of the water vapor barrier layer coating liquid A1.

## Comparative Example 2

## (Preparation of Water Vapor Barrier Layer Coating Liquid A5)

A water vapor barrier layer coating liquid A5 having a solid content concentration of 32% was obtained as in the water vapor barrier layer coating liquid A1 except that 5 parts (solid content) of the viscosity modifier (ethylene-modified polyvinyl alcohol) was changed to 0.45 parts (solid content) of a viscosity modifier (sodium polyacrylate, product name: ARONVIS MX, manufactured by TOAGOSEI Co., Ltd.).

A paper barrier base material was obtained as in Example 1 except that the water vapor barrier layer coating liquid A5 was used instead of the water vapor barrier layer coating liquid A1.

In Examples 1 and 2, both the stability of the coating liquid and the continuous operability were good. In Example 3, although the continuous operability was slightly inferior to those of Examples 1 and 2, Example 3 was sufficient for practical use.

In Comparative Example 1, although the stability of the coating liquid was good, the continuous operability was poor. In Comparative Example 2, both the stability of the coating liquid and the continuous operability were poor. None of Comparative Examples 1 and 2 was sufficient for practical use.

## Example 5

## (Preparation of Water Vapor Barrier Layer Coating Liquid a1)

To engineered kaolin (product name: Barrisurf HX, average particle size: 9.0 µm, aspect ratio: 80 to 100, manufactured by Imerys), polyacrylate soda was added (0.2% relative to the pigment) as a dispersant. The mixture was then dispersed in a Serie mixer to prepare a kaolin slurry having a solid content concentration of 60%. To 90 parts (solid content) of the kaolin slurry prepared above, 10 parts (solid

## 21

content) of talc (product name: TALCRON, manufactured by Specialty MINERALS Inc.) was added to prepare a pigment slurry having a solid content concentration of 50%.

Into the pigment slurry prepared above, 50 parts (solid content) of a styrene-acrylic copolymer emulsion (product name: X-511-374E, manufactured by Saiden Chemical Industry Co., Ltd.) and 50 parts (solid content) of an acrylic resin (product name: BARIASTAR ASN 1004, manufactured by Mitsui Chemicals, Inc.) relative to 100 parts (solid content) of the pigment were blended as water vapor barrier resins. Furthermore, a paraffin water repellent (product name: MYE-35G, wax-containing polyethylene emulsion, manufactured by Maruyoshi Chemical Co., Ltd.), a silicone surface-active agent (product name: SN-WET 125, manufactured by SAN NOPCO Limited), and a viscosity modifier (sodium polyacrylate, product name: ARONVIS MX, manufactured by TOAGOSEI Co., Ltd.) were blended such that the amounts of the paraffin water repellent, silicone surface-active agent, and viscosity modifier were 70 parts (solid content), 1.5 parts (solid content), and 0.05 parts (solid content), respectively, relative to 100 parts of the pigment. Thus, a water vapor barrier layer coating liquid a1 having a solid content concentration of 32% was obtained.

## (Preparation of Gas Barrier Layer Coating Liquid b1)

An aqueous solution of polyvinyl alcohol (product name: PVA117, manufactured by Kuraray Co., Ltd.) was prepared so as to have a solid content concentration of 12% to obtain a gas barrier layer coating liquid b1.

## (Production of Paper Barrier Base Material)

The water vapor barrier layer coating liquid a1 was applied to one surface of the obtained base paper with a

## 22

## Example 6

## (Preparation of Water Vapor Barrier Layer Coating Liquid a2)

5 A water vapor barrier layer coating liquid a2 having a solid content concentration of 32% was obtained as in the water vapor barrier layer coating liquid a1 except that the silicone surface-active agent (product name: SN-WET 125, manufactured by SAN NOPCO Limited) was blended such that the amount of the silicone surface-active agent was 2.0 parts (solid content) relative to 100 parts of the pigment.

10 A paper barrier base material was obtained as in Example 5 except that the water vapor barrier layer coating liquid a2 was used instead of the water vapor barrier layer coating liquid a1.

## Example 7

## (Preparation of Water Vapor Barrier Layer Coating Liquid a3)

15 A water vapor barrier layer coating liquid a3 having a solid content concentration of 32% was obtained as in the water vapor barrier layer coating liquid a1 except that the silicone surface-active agent (product name: SN-WET 125, manufactured by SAN NOPCO Limited) was blended such that the amount of the silicone surface-active agent was 3.0 parts (solid content) relative to 100 parts of the pigment.

20 A paper barrier base material was obtained as in Example 5 except that the water vapor barrier layer coating liquid a3 was used instead of the water vapor barrier layer coating liquid a1.

TABLE 2

|                                          |                                       | Example 5       | Example 6       | Example 7       |
|------------------------------------------|---------------------------------------|-----------------|-----------------|-----------------|
| Coating liquid                           |                                       | a1              | a2              | a3              |
| Water repellent                          |                                       | Paraffin        | Paraffin        | Paraffin        |
| Quantity of water repellent blended      | parts by weight (relative to pigment) | 70              | 70              | 70              |
| Surface-active agent                     |                                       | Silicone        | Silicone        | Silicone        |
| Quantity of surface-active agent blended | parts by weight (relative to pigment) | 1.5             | 2.0             | 3.0             |
| Viscosity modifier                       |                                       | Na polyacrylate | Na polyacrylate | Na polyacrylate |
| Quantity of viscosity modifier blended   | parts by weight (relative to pigment) | 0.05            | 0.05            | 0.05            |
| Coating color concentration              | %                                     | 32              | 32              | 32              |
| Spinnability                             | sec                                   | 0.10            | 0.10            | 0.10            |
| B-type viscosity                         | mPa · s                               | 200             | 200             | 200             |
| Static surface tension                   | mN/m                                  | 39              | 38              | 37              |
| Stability of coating liquid              |                                       | ○               | ○               | ○               |
| Continuous operability                   |                                       | ○               | ○               | ○               |
| Neck-in                                  |                                       | ○               | ○               | ○               |
| Water vapor permeability                 | g/m <sup>2</sup> · day                | 2.4             | 2.8             | 3.2             |
| Oxygen permeability                      | ml/m <sup>2</sup> · day               | 1.0             | 1.0             | 1.0             |

curtain coater at a coating speed of 300 m/min such that the coating quantity was 10 g/m<sup>2</sup> on a dry weight basis, and dried. Subsequently, the gas barrier layer coating liquid b1 was applied to the water vapor barrier layer coating liquid a1 with a curtain coater at a coating speed of 300 m/min such that the coating quantity was 5.0 g/m<sup>2</sup> on a dry weight basis. Thus, a paper barrier base material was obtained.

60 In Examples 5 to 7, both the stability of the coating liquid and the continuous operability were good. In Examples 5 and 6, neck-in did not occur during curtain coating, and the obtained paper barrier base material had both a good water vapor barrier property and a good gas barrier property. In 65 Example 7, although the vapor barrier property was slightly inferior to those of Examples 5 and 6, Example 7 was sufficient for practical use.

The invention claimed is:

1. A method for manufacturing a paper barrier base material, comprising:

a step of applying a water vapor barrier layer coating liquid that contains at least a water vapor barrier resin and a pigment onto a paper base material by a curtain coating method to form a water vapor barrier layer, wherein the water vapor barrier layer coating liquid has a spinnability of 0.07 seconds or more and 0.4 seconds or less at a solid content concentration of 32% by weight and a temperature of 25° C., wherein the water vapor barrier layer coating liquid contains a viscosity modifier, and wherein the viscosity modifier contains ethylene-modified polyvinyl alcohol.

2. The method for manufacturing a paper barrier base material according to claim 1, wherein a blending quantity of the ethylene-modified polyvinyl alcohol is 1% by weight or more and 20% by weight or less in terms of solid content relative to the pigment in the water vapor barrier layer coating liquid.

3. A method for manufacturing a paper barrier base material, comprising:

a step of applying a water vapor barrier layer coating liquid that contains at least a water vapor barrier resin and a pigment onto a paper base material by a curtain coating method to form a water vapor barrier layer, wherein the water vapor barrier layer coating liquid has a spinnability of 0.07 seconds or more and 0.4 seconds or less at a solid content concentration of 32% by weight and a temperature of 25° C., wherein the water vapor barrier layer coating liquid contains a viscosity modifier, and wherein the viscosity modifier contains sodium polyacrylate.

4. The method for manufacturing a paper barrier base material according to claim 3, wherein a blending quantity of the sodium polyacrylate is 0.01% by weight or more and 0.5% by weight or less in terms of solid content relative to the pigment in the water vapor barrier layer coating liquid.

5. The method for manufacturing a paper barrier base material according to claim 3, wherein the water vapor barrier layer coating liquid further contains a water repellent and a surface-active agent and has a static surface tension of 40 mN/m or less at a solid content concentration of 32% by weight and a temperature of 25° C.

6. The method for manufacturing a paper barrier base material according to claim 5, wherein the water repellent contains a paraffin water repellent.

7. The method for manufacturing a paper barrier base material according to claim 5, wherein a blending quantity of the water repellent is 20 parts by weight or more and 100 parts by weight or less in terms of solid content relative to 100 parts by weight of the pigment in the water vapor barrier layer coating liquid.

8. The method for manufacturing a paper barrier base material according to claim 5, wherein a blending quantity of the surface-active agent is 0.3 parts by weight or more and 3.0 parts by weight or less in terms of solid content relative to 100 parts by weight of the pigment in the water vapor barrier layer coating liquid.

9. The method for manufacturing a paper barrier base material according to claim 3, wherein the water vapor barrier layer coating liquid has a solid content concentration of 25% by weight or more and 45% by weight or less.

10. The method for manufacturing a paper barrier base material according to claim 3, comprising a step of applying a gas barrier layer coating liquid onto the water vapor barrier layer to form a gas barrier layer.

11. The method for manufacturing a paper barrier base material according to claim 1, wherein the water vapor barrier layer coating liquid further contains a water repellent and a surface-active agent and has a static surface tension of 40 mN/m or less at a solid content concentration of 32% by weight and a temperature of 25° C.

12. The method for manufacturing a paper barrier base material according to claim 1, wherein the water vapor barrier layer coating liquid has a solid content concentration of 25% by weight or more and 45% by weight or less.

13. The method for manufacturing a paper barrier base material according to claim 1, comprising a step of applying a gas barrier layer coating liquid onto the water vapor barrier layer to form a gas barrier layer.

14. The method for manufacturing a paper barrier base material according to claim 2, wherein the water vapor barrier layer coating liquid further contains a water repellent and a surface-active agent and has a static surface tension of 40 mN/m or less at a solid content concentration of 32% by weight and a temperature of 25° C.

15. The method for manufacturing a paper barrier base material according to claim 2, wherein the water vapor barrier layer coating liquid has a solid content concentration of 25% by weight or more and 45% by weight or less.

\* \* \* \* \*